# EUROPEAN PATENT SPECIFICATION

(11) **EP 3 572 534 B1**
(45) Date of publication and mention of the grant of the patent: **28.04.2021**
(21) Application number: 18741544.3
(22) Date of filing: 10.01.2018
(51) Int. Cl.: C21C 7/00, C21C 7/04, C21C 7/072, C21C 7/076, C21C 7/064

(54) **DESULFURIZATION PROCESSING METHOD OF MOLTEN STEEL, AND DESULFURIZATION AGENT**
ENTSCHWEFELUNGSBEHANDLUNGSVERFAHREN FÜR GESCHMOLZENEN STAHL UND ENTSCHWEFELUNGSMITTEL
PROCEDE DE TRAITEMENT DE DÉSULFURATION D'ACIER FONDU ET AGENT DE DÉSULFURATION

(30) Priority: 19.01.2017 JP 2017007209
(43) Date of publication of application: 27.11.2019
(73) Proprietor: JFE Steel Corporation, Tokyo 100-0011 (JP)
(72) Inventor: FUJII, Yusuke, Tokyo 100-0011 (JP); NAKAI, Yoshie, Tokyo 100-0011 (JP); MASAKI, Hideya, Tokyo 100-0011 (JP); KIKUCHI, Naoki, Tokyo 100-0011 (JP)
(74) Representative: Hoffmann Eitle
(86) International application number: PCT/JP2018/000280
(87) International publication number: WO 2018/135344

(56) References cited:
- EP-A1- 2 434 025
- WO-A1-2010/026775
- WO-A1-2017/018263
- WO-A1-2017/018263
- JP-A- S6 256 509
- JP-A- S6 256 509
- JP-A- H11 221 432
- JP-A- H11 221 432
- JP-A- S62 283 847
- JP-A- 2004 225 059
- JP-A- 2008 063 647
- JP-A- 2009 108 344
- JP-A- 2009 108 344
- JP-A- 2017 071 853
- JP-A- 2017 071 853
- JP-A- 2017 071 854
- JP-A- 2017 071 854

## Description

### Field

The present invention relates to a desulfurization processing method of molten steel, a desulfurization agent and the use of said desulfurization agent in desulfurization of molten steel.

### Background

Recently, high purity steel manufacturing has been highly demanded for enhancing material characteristics along with adding high value to steel and an increase in use of steel materials, for example. Particularly, a demand has been highly increased for ultra low sulfur steel having a low content of sulfur, which is an element that reduces toughness of steel materials. In melting manufacturing processes of steel materials, desulfurization processing at a molten pig iron stage and desulfurization processing at a molten steel stage are available. Steel materials are typically subjected to only the desulfurization processing at the molten pig iron stage when manufactured by being melted. In the melting manufacturing processes of ultra low sulfur steel such as high-grade electromagnetic steel plates and line pipe steel materials, it is insufficient to perform only the desulfurization processing at the molten pig iron stage. It is, thus, necessary to perform the desulfurization processing at the molten steel stage in addition to the desulfurization processing at the molten pig iron stage.

The desulfurization processing at the molten steel stage is typically performed by a ladle refining method such as an ASEA-SKF method, a VAD method, or an LF method. The ladle reining method includes an arc heating means to heat molten steel and a stirring means to stir molten steel, and further includes a blowing means to blow powder such as flux or alloy powder to molten steel. In the ladle refining method, a desulfurization agent is added into a ladle holding molten steel manufactured by being melted by decarburization refining in a converter, the molten steel and the desulfurization agent are stirred and mixed with each other or subjected to arc heating, thereby causing the desulfurization agent to form slag, and a slag-metal reaction occurs between the slag formed by slag formation of the desulfurization agent and the molten steel to transfer sulfur in the molten steel to the slag.

The used desulfurization agent contains CaO (quicklime) as a major component and Al₂O₃ (alumina), CaF₂ (fluorite), and the like, which are added for the purpose of lowering a melting point of the desulfurization agent. For achieving effective desulfurization reaction in the desulfurization processing method by the ladle refining method, it is important to cause the added desulfurization agent to rapidly form slag and to increase a contact area between the slag formed by the slag formation of the desulfurization agent and the metal by increasing stirring strength. The desulfurization agent is typically added to molten steel in the ladle by being placed on the molten steel. It takes a long time that the desulfurization agent forms slag in any case where the desulfurization agent forms slag by arc heating or by being stirred and mixed with the molten steel after the desulfurization agent is added.

Patent Literature 1 discloses a method of desulfurizing molten steel in which flux, a mixture of quicklime, alumina, and fluorite, is added and bubbling processing is performed such that a slag composition after the desulfurization processing satisfies that CaO/Al₂O₃ ≥ 1.5 mass% and CaF₂ ≥ 5 mass%. Patent Literature 2 discloses a method in which pre-melt flux (preliminarily mixed or uniformly dissolved) of CaO-Al₂O₃ or pre-melt flux of CaO-Al₂O₃-CaF₂ is used for promoting the slag formation of the desulfurization agent. As for enhancing stirring strength of molten steel, Patent Literatures 3, 4, and 5 disclose a method in which stirring gas mixed with flux is blown, as a means to enhance the stirring strength without increasing a stirring gas flow rate.

### Citation List

### Patent Literature

Patent Literature 1: Japanese Patent Application Laid-open No. H08-260025
Patent Literature 2: Japanese Patent Application Laid-open No. H09-217110
Patent Literature 3: Japanese Patent Application Laid-open No. S61-91318
Patent Literature 4: Japanese Patent Application Laid-open No. S61-281809
Patent Literature 5: Japanese Patent Application Laid-open No. 2000-234119

JP 2009-108344 discloses a desulfurization agent used when performing desulfurization of molten pig iron or molten steel, wherein the desulfurization agent is a powder containing quicklime having an average particle size of 200 pm or less and an average core diameter of 5 to 40 pm on the surface of the powder.

WO 2017/018263 A1 discloses a desulfurization processing method of molten pig iron by adding a desulfurization agent containing quicklime into a ladle holding the molten pig iron, wherein the desulfurization agent contains powdery quicklime, where a sum of volumes of pores having a pore diameter ranging from 0.5 pm to 10 pm (inclusive) in the quicklime is equal to or larger than 0.1 mL/g, the quicklime has an average particle size of 210 pm or more and 500 pm or less.

### Summary

### Technical Problem

The method described in Patent Literature 1, however, has a problem in that, when a desulfurization agent containing CaF₂ is used, refractory forming the ladle is heavily melted and eroded by CaF₂ in the produced slag, thereby significantly shortening a life-span of the ladle. The method described in Patent Literature 2 has a problem in that the pre-melt flux is very expensive, thereby increasing processing cost. The desulfurization agent containing CaF₂ has the same problem as described above.

The method described in Patent Literatures 3, 4, and 5, has a limit for a flux blowing amount with respect to a blowing gas rate (a solid-gas ratio has a limit ranging from 5 to 30 kg/kg). The method, thus, has a limit for increasing stirring strength. When a stirring gas flow rate is increased, a surface of molten steel in the ladle is heavily disturbed (waved). As a result, a problem arises in that splashes occur and metal sticks to a lid of the ladle, or another problem arises in that electrodes and molten steel are shorted, for example, to cause unstable arc, thereby making it difficult to perform arc heating.

The invention is made in view of above problems, and aims to provide a desulfurization processing method of molten steel and a desulfurization agent that can efficiently perform desulfurization processing without using CaF₂ and pre-melt flux.

### Solution to Problem

To solve the problem and achieve the object, a desulfurization processing method of molten steel , a desulfurization agent and the use of a desulfurization agent are described in the claims.

Moreover, in the desulfurization processing method of molten steel according to the present invention, argon gas is blown into the ladle such that an oxygen concentration in the ladle is equal to or smaller than 15%. Advantageous Effects of Invention

The desulfurization processing method of molten steel and the desulfurization agent according to the invention can efficiently perform desulfurization processing without using CaF₂ and pre-melt flux.

### Brief Description of Drawings

FIG. 1 is a schematic diagram of a side surface of an LF facility used when the invention is implemented.
FIG. 2 is a diagram illustrating slagging ratios in invention examples and comparative examples.

### Description of Embodiment

The inventors of the invention have earnestly studied for solving the problems described above by focusing attention on a particle size and a pore diameter of caustic lime and molten steel components. More specifically, the inventors of the invention have performed various experiments and researches for the purpose of causing flux added as a desulfurization agent to rapidly form slag to achieve efficient desulfurization processing without using CaF₂ as a part of the desulfurization agent when low sulfur steel having a sulfur concentration equal to or smaller than 0.0030 mass% is manufactured by being melted by desulfurization processing by a ladle refining method using a desulfurization agent having a CaO containing material as a major constituent material.

As a result, the inventors of the invention have found that the temperature of molten steel when flux is added, a sol. Al concentration, and the particle size and the pore diameter of caustic lime are important in order to promote flux added as a desulfurization agent to form slag. The temperature of molten steel is determined by the temperature of molten steel when the molten steel is tapped from a converter. As the temperature of the molten steel when the molten steel is tapped is increased, the refractory of the converter is increasingly melted and eroded, thereby causing processing cost to be increased. An immoderate increase in tapping temperature is, thus, inadvisable.

The inventors of the invention have found that the desulfurization processing can be performed highly efficiently using a powder desulfurization agent containing quicklime as a major component and the quicklime satisfies that a sum of volumes of pores having a pore diameter ranging from 0.5 to 10 µm in all of the pores included in the quicklime is equal to or larger than 0.1 mL/g. The inventors of the invention, thus, have conceived the invention. The pore diameter distribution of quicklime was measured by the following method.

As pretreatment, quicklime was dried at a constant temperature of 120 °C for 4 hours. Using Micromeritics autopore IV 9520, a pore diameter distribution of dried quicklime having a pore diameter ranging from approximately 0.0036 to 200 µm was obtained by a mercury intrusion method, and a cumulative pore volume curve was calculated. In addition, a sum of volumes of pores having a pore diameter ranging from 0.5 to 10 µm was obtained from the calculated cumulative pore volume curve.

The pore diameter was calculated using Washburn's equation represented in the following formula (3). In formula (3), P is the pressure, D is the pore diameter, σ is the surface tension (= 480 dynes/cm) of mercury, θ is the contact angle (= 140 degrees) between mercury and the specimen.$P \times D = - 4 \times σ \times cos θ$

Molten pig iron tapped from a blast furnace is received by a hot metal transfer vessel such as a hot metal ladle or a torpedo car, and transferred to a converter in which decarburization refining is performed as the next process. Typically, during the transportation, hot metal pretreatment such as desulfurization processing and dephosphorization processing are performed on molten pig iron. The invention is the technique to manufacture low sulfur steel. The desulfurization processing is, thus, performed. Even when the dephosphorization processing is not required in accordance with the compositional standard of the low sulfur steel, the dephosphorization processing is performed to prevent rephosphorization from converter slag in desulfurization processing after tapping from the converter.

The decarburization refining is performed on the molten pig iron on which the desulfurization processing and the dephosphorization processing are performed, and resulting molten steel is tapped to the ladle. In the decarburization refining in the converter, a little amount of quicklime (CaO) and a little amount of dolomite (MgCO₃-CaCO₃), or calcined dolomite (MgO-CaO) is used as flux, and the flux forms slag in the converter (hereinafter described as the "converter slag"), because the desulfurization processing and the dephosphorization processing are already performed on the molten pig iron. The converter slag has a role to promote dephosphorization reaction of the molten pig iron. The dephosphorization processing is, however, already performed on the molten pig iron. The main role of converter slag is, thus, prevention of occurrence of iron splashes in blowing refining and melting and erosion of the lining refractory of the converter.

At the last stage of tapping, the converter slag is mixed into the molten steel and flows into the ladle. Slag flow-out prevention measures, which are typically taken, are performed to prevent the flow out of the converter slag. It is, however, difficult to perfectly prevent the converter slag from being flowed out even when the slag flow-out prevention measures are taken. Some amount of converter slag is mixed into the molten steel in the ladle and flows out from the converter. After tapping, the converter slag that is mixed into the molten steel and flows into the ladle may be removed from the ladle. The converter slag may, however, not be removed because SiO₂ component in the converter slag contributes to the slag formation of a CaO containing material added later as the desulfurization agent.

In order to form CaO-MgO-Al₂O₃-SiO₂ desulfurization slag having a certain composition in the ladle, a CaO containing material, a MgO containing material, an Al₂O₃ containing material, and a SiO₂ containing material are added into the ladle as flux. As described above, MgO has a lower desulfurization ability than that of CaO, the MgO containing material may not be added. Metallic Al is added into the ladle for deoxidation of the molten steel and reduction of the slag (reduction of Fe oxides and Mn oxides in the slag).

Those materials may be added into a facility in later process that performs desulfurization processing by any of an ASEA-SKF method, a VAD method, and an LF method. From a point of view of promoting the slag formation of CaO, those materials are preferably added into the ladle at tapping from the converter to the ladle or just after the tapping. It is preferable for quicklime added just after the tapping that a sum of volumes of pores having a pore diameter ranging from 0.5 to 10 µm in all of the pores included in the quicklime is equal to or larger than 0.1 mL/g, and the quicklime contains particles 90% or more of which have a particle diameter ranging from 1 to 30 mm.

Respective additive amounts of the CaO containing material, the MgO containing material, metallic Al, the Al₂O₃ containing material, and the SiO₂ containing material are determined, by considering a mass and a component composition of converter slag flowed into the ladle, such that the composition of the slag produced in the ladle after the slag formation of the added flux, i.e., the slag formed from the flux and the converter slag, satisfies that the SiO₂ content is in a range from 5 to 15 mass% and a value of [(mass% CaO) + (mass% MgO)]/(mass% Al₂O₃) is in a range from 1.5 to 3.0, and, preferably, the value of [(mass% CaO) + (mass% MgO)]/(mass% Al₂O₃) is in a range from 1.8 to 2.5.

In this case, the respective additive amounts are more preferably determined such that a value of (mass% MgO)/(mass% CaO) of the produced slag is equal to or smaller than 0.10. Those materials are added into the ladle by the determined additive amounts. All of the additive amount of metallic Al does not become Al₂O₃. Some amount of metallic Al is dissolved and remains in the molten steel. A ratio of Al₂O₃ in slag to Al dissolved in molten steel is obtained preliminarily by an experiment. The additive amount of metallic Al is set on the basis of the ratio. No CaF₂ is added.

In the invention, "the composition of the slag in the ladle after the desulfurization processing is adjusted to the composition that does not substantially contain CaF₂" means that the slag composition of after the desulfurization processing is adjusted without using a fluorine compound such as CaF₂ as a slag formation accelerator of CaO, and even when fluorine that is unavoidably mixed into the used CaO containing material and Al₂O₃ containing material, for example, and brought into the ladle is present in the slag after the desulfurization processing, the slag in the ladle is defined that the slag substantially does not contain CaF₂.

As for the CaO containing material to be added, quicklime (CaO), limestone (CaCO₃), slaked lime (Ca(OH)₂), dolomite (MgCO₃-CaCO₃), and calcined dolomite (MgO-CaO) are used, for example. As for the MgO containing material to be added, magnesia clinker (MgO), dolomite (MgCO₃-CaCO₃), and calcined dolomite (MgO-CaO) are used, for example.

It is preferable for a particle size of caustic lime that an average particle diameter of the caustic lime is in a range from 1 to 30 mm from a point of view of a reaction efficiency and an addition yield. From a point of view of reducing an amount sucked in an exhaust system, an amount of fine powder is preferably small. An amount of caustic lime having an average particle diameter equal to or larger than 30 mm is, thus, preferably small. The measuring method of the average particle diameter is as follows. One kilogram of a desulfurization agent was collected. The collected desulfurization agent was sieved into nine classes, i.e., equal to or smaller than 500 µm, 500 µm to 1 mm, 1 to 5 mm, 5 to 10 mm, 10 to 15 mm, 15 to 20 mm, 20 to 25 mm, 25 to 30 mm, and equal to or larger than 30 mm. The average particle diameter was obtained by calculating the weight ratio represented in the following formula (4).${D}_{a} = \frac{{\sum }_{i} \left({w}_{i}\right)}{\sum \left({w}_{i}/{d}_{i}\right)}$
*Dₐ : average particle diameter (mm)*
*dᵢ* : *average particle diameter (sieve mesh median) (mm)*
*in each particle diameter range*
*wᵢ : slag weight (kg) on each sieve*

As for the Al₂O₃ containing material, aluminum dross (contains 20 to 70 mass% metallic Al and main component of the balance is Al₂O₃) , bauxite (Al₂O₃·2H₂O), and calcined alumina (Al₂O₃) are used, for example. Aluminum dross can be used as alternative of metallic Al. As for the SiO₂ containing material, silica sand (SiO₂) and wollastonite (CaO-SiO₂) are used, for example. When the mass of the converter slag flowed in the ladle is large, the SiO₂ containing material may not be required to be added. The MgO containing material may not be required to be added when the slag composition satisfies that a value of [(mass% CaO) + (mass% MgO)]/(mass% Al₂O₃) is in a range from 1.5 to 3.0, preferably in a range 1.8 to 2.5 without addition of the MgO containing material.

The ladle holding the molten steel is transferred to the facility that performs the desulfurization processing by any of the ASEA-SKF method, the VAD method, and the LF method, and the desulfurization processing is performed on the molten steel by the facility. In the invention, the desulfurization processing is performed by an LF facility as an example. FIG. 1 is a schematic diagram of a side view of the LF facility used when the invention is implemented. FIG. 1 illustrates an LF facility 1, a ladle 2, an elevating lid 3, arc heating electrodes 4, submerged lances 5 and 6, bottom-blowing porous bricks 7 and 8, molten steel 9, slag 10, a row material supply chute 11, and an Ar gas introduction pipe 12.

In the LF facility 1, the ladle 2 that contains the molten steel 9 and is mounted on a traveling carriage (not illustrated) is disposed at a certain position just under the lid 3. The lid 3 is moved downward to be tightly in contact with the upper end of the ladle 2. While the contact is kept, Ar gas is supplied from the Ar gas introduction pipe 12, resulting in a space surrounded by the ladle 2 and the lid 3 becoming Ar gas atmosphere. Ar gas is preferably blown from piping provided on the periphery of the furnace lid such that an oxygen concentration in the ladle 2 is equal to or smaller than 15%. The reduction of the oxygen concentration in the ladle 2 makes it possible to reduce an amount of Al lost by reaction with oxygen in the air in the LF processing. The flow rate of Ar gas blown from the ladle 2 preferably satisfies that a value of πL²/4Q is in a range from 50 to 150 (m/min) and more preferably 70 to 100 (m/min). L is the diameter (m) of the ladle and Q is the flow rate of Ar gas (Nm³/min). When the flow rate of Ar gas is small, the oxygen concentration is not sufficiently reduced. In contrast, when the flow rate of Ar gas is too large, the molten steel temperature is caused to be reduced.

When the CaO containing material, the MgO containing material, metallic Al, the Al₂O₃ containing material, and the SiO₂ containing material are not preliminarily added into the ladle 2, and when the additive amounts of those materials are insufficient, the flux containing those materials and metallic Al are supplied into the ladle 2 via the row material supply chute 11. Metallic Al is preferably added within 10 minutes after start of the desulfurization processing such that the following formula (5) is satisfied. It is, thus, preferable for promoting the desulfurization processing that metallic Al is added in accordance with the Al concentration after tapping from the converter to increase the Al concentration in molten steel.$\left({\left[sol.Al\right]}_{1}-{\left[sol.Al\right]}_{2}+0.05\right) \leq {W}_{Al} \leq \left({\left[sol.Al\right]}_{1}-{\left[sol.Al\right]}_{2}+0.1\right)$
[*sol.Al*]₁ *: Al concentration standard upper limit (mass%)*
*in steel grade to be manufactured by being melted*
[*sol.Al*]₂ *: Al concentration (mass%) in molten steel after tapping from converter*
*W_{Al} : amount (kg*/*t) of Al supplied within 10 minutes*
*after start of ladle desulfurization processing*

Then, the electrodes 4 are energized to generate arc, if necessary, to heat the molten steel 9 and to cause the added flux to form slag. Thereafter, the submerged lance 5 or 6 is immersed into the molten steel 9 and then Ar gas serving as a stirring gas is blown into the molten steel 9 from at least one of the submerged lances 5 and 6, or the bottom-blowing porous bricks 7 and 8 to stir the molten steel 9. As a result of stirring the molten steel 9, the flux is mixed with the molten steel 9, thereby causing the flux to form slag. As a result, slag 10 is produced.

The produced slag 10 is stirred and mixed with the molten steel 9 as a result of stirring of the molten steel 9. As a result, a slag-metal reaction occurs between the molten steel 9 and the slag 10 and, thus, a desulfurization reaction occurs in which sulfur in the molten steel 9 transfers into the slag. From a point of view of promoting the desulfurization reaction, as described above, one or more kinds of Ca alloy powder, metallic Mg powder, and Mg alloy powder are preferably blown into the molten steel 9 together with Ar gas from the submerged lances 5 and 6, or, at least one period in the desulfurization processing, blowing of the stirring gas from the submerged lances 5 and 6 and blowing of the stirring gas from the bottom-blowing porous bricks 7 and 8 are preferably performed simultaneously.

As for the Ca alloy powder, Ca-Si alloy powder and Ca-Al alloy powder are used, for example. As for the Mg alloy powder, Mg-Al-Zn alloy powder and Mg-Si-Fe alloy powder are used, for example. The particle diameters of those metallic powder are not limited to specific diameters as long as those metallic powder can be added by being blown. From a point of view of keeping a reaction interfacial area, the maximum particle diameter is preferably equal to or smaller than 1 mm. When the sulfur concentration in the molten steel 9 becomes equal to or smaller than 0.0010 mass%, blowing Ar gas into the molten steel 9 stops to end the desulfurization processing. When the temperature of the molten steel 9 is lower than a target temperature at the end of the desulfurization processing, arc heating is performed. When the composition of the molten steel 9 is not in a target range, an alloy iron and metals for composition adjustment are supplied via the row material supply chute 11. After the completion of the desulfurization processing, degassing refining is performed by an RH vacuum degassing apparatus, for example. Thereafter, a strip cast slab is casted by a continuous casting machine.

As described above, in the invention, the slag composition after the desulfurization processing is adjusted such that the SiO₂ content is in a range from 5 to 15 mass% in the desulfurization processing of the molten steel 9 by the ladle refining method using the desulfurization agent containing the CaO containing material as the major constituent material. SiO₂, thus, functions as the slagging accelerator to promote the slag formation of CaO. In addition, the slag composition after the desulfurization processing is adjusted such that a value of [(mass% CaO) + (mass% MgO)]/(mass% Al₂O₃) is in a range from 1.5 to 3.0, thereby causing the slag 10 to have high desulfurization ability. As a result, the desulfurization processing can be efficiently performed on the molten steel 9 without using CaF₂ as a part of the desulfurization agent and pre-melt flux as the desulfurization agent. The above description is an example where the invention is implemented using the LF facility. The invention can also be applied to an ASEA-SKF facility and a VAD facility according to the manner as described above.

### [First example]

Molten pig iron tapped from a blast furnace was subjected to the desiliconization processing, the desulfurization processing, and the dephosphorization processing. The processed molten pig iron was, then, charged into a converter to be subjected to the decarburization refining. As a result, obtained was approximately 250 tons of molten steel having a carbon concentration ranging from 0.05 to 0.09 mass%, a sulfur concentration ranging from 0.0041 to 0.0043 mass%, and a phosphorous concentration ranging from 0.004 to 0.010 mass%. After tapping, the converter slag flowed in a ladle was not discharged. Metallic Al, quicklime, lightly calcined dolomite, and aluminum dross were added into the ladle, and the ladle was transferred to the LF facility illustrated in FIG. 1. The desulfurization processing was performed for approximately 30 minutes in such a manner that the molten steel was stirred by blowing Ar gas at 2000 NL/min from the submerged lances into the molten steel while the arc heating was performed by the electrodes immersed in the slag so as to achieve a target sulfur concentration equal to or smaller than 0.0024%.

Table 1 illustrates the sulfur concentrations (chemical analysis values) before and after the desulfurization processing and the desulfurization ratios in respective desulfurization tests. The remarks column in Table 1 illustrates "invention examples", which are the tests according to the invention, and "comparative examples", which are the tests other than those according to the invention. The desulfurization ratio is the value of a ratio of a difference in sulfur concentration in the molten steel before and after the desulfurization processing to a sulfur concentration in the molten steel before the desulfurization processing and the value is expressed by percentage. The desulfurization evaluation "Good" means that the sulfur concentration in the molten steel after the desulfurization processing was equal to or smaller than 0.0024% while the desulfurization evaluation "Poor" means that the sulfur concentration in the molten steel after the desulfurization processing exceeded 0.0024%.

**Table 1**

| Test No. | Sum of volumes of pores 0.5-10 µm | Average particle diameter | [S]Component change | | | Desulfurization evaluation | Remarks |
|---|---|---|---|---|---|---|---|
| | | | Before processing [S] | After processing [S] | Desulfurization ratio | | |
| | mL/g | mm | Mass [%] | Mass [%] | [%] | - | |
| 1 | 0.03 | 10 | 0.0042 | 0.0028 | 33.3 | Poor | Comparative example |
| 2 | 0.06 | 10 | 0.0043 | 0.0027 | 37.2 | Poor | Comparative example |
| 3 | 0.09 | 10 | 0.0041 | 0.0025 | 39.0 | Poor | Comparative example |
| 4 | 0.15 | 10 | 0.0042 | 0.0021 | 50.0 | Good | Example |
| 5 | 0.2 | 10 | 0.0042 | 0.0019 | 54.8 | Good | Example |
| 6 | 0.2 | 0.5 | 0.0044 | 0.0022 | 50.0 | Good | Reference Example |
| 7 | 0.2 | 0.8 | 0.0041 | 0.0020 | 51.2 | Good | Reference Example |
| 8 | 0.2 | 1.5 | 0.0043 | 0.0018 | 58.1 | Good | Example |
| 9 | 0.2 | 3 | 0.0043 | 0.0016 | 62.8 | Good | Example |
| 10 | 0.2 | 5 | 0.0042 | 0.0016 | 61.9 | Good | Example |
| 11 | 0.2 | 15 | 0.0041 | 0.0015 | 63.4 | Good | Example |
| 12 | 0.2 | 25 | 0.0043 | 0.0014 | 67.4 | Good | Example |
| 13 | 0.2 | 28 | 0.0042 | 0.0016 | 61.9 | Good | Example |
| 14 | 0.2 | 32 | 0.0043 | 0.0017 | 60.5 | Good | Reference Example |
| 15 | 0.2 | 40 | 0.0042 | 0.0019 | 54.8 | Good | Reference Example |

Table 1 also illustrates the test levels and the results. In the comparative examples (test numbers 1 to 3), in which the sum of volumes of pores having a pore diameter ranging from 0.5 to 10 µm is inadequate, the desulfurization ratios were lower than those in the invention examples (test numbers 4, 5 and 8 to 13). In the invention examples having test levels in each of which the average particle diameter of quicklime is in a range from 1 to 30 mm, slag formation was promoted and the desulfurization ratio of molten steel were higher.

### [Second example]

Molten pig iron tapped from a blast furnace was subjected to the desiliconization processing, the desulfurization processing, and the dephosphorization processing. The processed molten pig iron was, then, charged into a converter to be subjected to the decarburization refining. As a result, obtained was approximately 250 tons of molten steel having a carbon concentration ranging from 0.05 to 0.09 mass%, a sulfur concentration ranging from 0.0041 to 0.0043 mass%, and a phosphorous concentration ranging from 0.004 to 0.010 mass%. After tapping, the converter slag flowed in a ladle was not discharged. Metallic Al, quicklime, lightly calcined dolomite, and aluminum dross were added into the ladle, and the ladle was transferred to the LF facility illustrated in FIG. 1. The desulfurization processing was performed for approximately 30 minutes in such a manner that the molten steel was stirred by blowing Ar gas at 500 to 2000 NL/min from the submerged lances into the molten steel while the arc heating was performed by the electrodes immersed in the slag so as to achieve a target sulfur concentration equal to or smaller than 0.0024%.

Table 2 illustrates the sulfur concentrations (chemical analysis values) before and after the desulfurization processing and the desulfurization ratios in respective desulfurization tests. The desulfurization evaluation "Good" means that the sulfur concentration in the molten steel after the desulfurization processing was equal to or smaller than 0.0024%.

**Table 2**

| Test No. | Stirring power density | Slagging ratio 5 min. after start of LF processing | [S]Component change | | | Desulfurization evaluation | Remarks |
|---|---|---|---|---|---|---|---|
| | | | Before processing [S] | After processing [S] | Desulfurization ratio | | |
| | [W/t] | [%] | Mass [%] | Mass [%] | [%] | - | - |
| 16 | 10 | 35 | 0.0042 | 0.0019 | 54.8 | Good | Example |
| 17 | 15 | 50 | 0.0042 | 0.0018 | 57.1 | Good | Example |
| 18 | 27 | 57 | 0.0041 | 0.0018 | 56.1 | Good | Example |
| 19 | 35 | 68 | 0.0042 | 0.0018 | 57.1 | Good | Example |
| 20 | 45 | 85 | 0.0042 | 0.0017 | 59.5 | Good | Example |
| 21 | 55 | 94 | 0.0042 | 0.0017 | 59.5 | Good | Example |
| 22 | 74 | 100 | 0.0042 | 0.0017 | 59.5 | Good | Example |
| 23 | 100 | 100 | 0.0043 | 0.0015 | 65.1 | Good | Example |
| 24 | 135 | 100 | 0.0041 | 0.0014 | 65.9 | Good | Example |
| 25 | 158 | 100 | 0.0042 | 0.0013 | 69.0 | Good | Example |
| 26 | 167 | 100 | 0.0042 | 0.0012 | 71.4 | Good | Example |
| 27 | 185 | 100 | 0.0044 | 0.0011 | 75.0 | Good | Example |

Table 2 also illustrates the test levels and the results. It was found that with an increase in stirring power, the slagging ratio after 5 minutes from start of the LF processing and the desulfurization ratio were increased. It was found that high slagging ratio and desulfurization ratio were obtained because the stirring power density satisfies the following formula (6).$ε = 6.183 \times \frac{Q \times {T}_{1}}{W} \times \left(ln\left(1+\frac{h}{1.02 \times {10}^{- 4} \times P}\right)+\left(1-\frac{{T}_{g}}{{T}_{l}}\right)\right) \geq 100$
ε : *stirring power density (W*/*t) of gas stirring molten steel,*
*Q* : *gas flow rate (Nm³*/*min),*
*W* : *molten steel amount (t),*
*Tₗ* : *molten steel temperature (°C),*
*T_{g}* : *gas temperature (°C),*
*h* : *bath depth (m), P : ambient pressure (Pa)*

### [Third example]

FIG. 2 is a diagram illustrating the slagging ratios of the invention examples and the comparative examples. The invention examples used quicklime satisfying that the quicklime has a particle diameter equal to or smaller than 20 mm and the sum of the volumes of pores having a pore diameter ranging from 0.5 to 10 µm is 0.2 mL/g. The comparative examples used quicklime satisfying that the quicklime has a particle diameter equal to or smaller than 20 mm and the sum of the volumes of pores having a pore diameter ranging from 0.5 to 10 µm is 0.03 mL/g. As illustrated in FIG. 2, it was found that slagging was more promoted in the invention examples than that in the comparative examples even at the identical stirring power density (135 W/t).

### [Fourth example]

Molten pig iron tapped from a blast furnace was subjected to the desiliconization processing, the desulfurization processing, and the dephosphorization processing. The processed molten pig iron was, then, charged into a converter to be subjected to the decarburization refining. As a result, obtained was approximately 250 tons of molten steel having a carbon concentration ranging from 0.05 to 0.09 mass%, a sulfur concentration ranging from 0.0041 to 0.0044 mass%, and a phosphorous concentration ranging from 0.004 to 0.010 mass%. After tapping, the converter slag flowed in a ladle was not discharged. Metallic Al, quicklime, lightly calcined dolomite, and aluminum dross were added into the ladle, and the ladle was transferred to the LF facility illustrated in FIG. 1. The LF processing used quicklime satisfying that the quicklime has a particle diameter equal to or smaller than 20 mm and the sum of the volumes of pores having a pore diameter ranging from 0.5 to 10 µm is 0.2 mL/g.

Table 3 illustrates the sulfur concentrations (chemical analysis values) before and after the desulfurization processing and the desulfurization ratios in respective desulfurization tests. [sol.Al]₁ is the upper limit value (mass%) of an Al concentration standard of a steel grade to be manufactured by being melted and [sol.Al]₂ is the Al concentration (mass%) in the molten steel after tapping from the converter. The desulfurization evaluation "Good" means that the sulfur concentration in the molten steel after the desulfurization processing was equal to or smaller than 0.0024%.

**Table 3**

| Test No. | [sol.Al] ₁ | [sol.Al]₂ | Left side of Formula (5) | Right side of Formula (5) | Wₐₗ | [sol.Al]₃ | RH processing time | [S]Component change | | | Desulfurization evaluation | Remarks |
|---|---|---|---|---|---|---|---|---|---|---|---|---|
| | | | | | | | | Before processing [S] | After processing [S] | Desulfurization ratic | | |
| | % | % | kg/t | kg/t | kg/t | % | min | Mass [%] | Mass [%] | [%] | - | |
| 28 | 0.050 | 0.023 | 0.77 | 1.27 | 1 | 0.039 | 30 | 0.0042 | 0.0011 | 73.8 | Good | Example |
| 29 | 0.050 | 0.025 | 0.75 | 1.25 | 1.1 | 0.043 | 29 | 0.0043 | 0.0011 | 74.4 | Good | Example |
| 30 | 0.050 | 0.026 | 0.74 | 1.24 | 1.2 | 0.047 | 31 | 0.0041 | 0.0010 | 75.6 | Good | Example |
| 31 | 0.050 | 0.024 | 0.76 | 1.26 | 1.3 | 0.051 | 36 | 0.0042 | 0.0009 | 78.6 | Good | Example |
| 32 | 0.050 | 0.025 | 0.75 | 1.25 | 1.4 | 0.055 | 39 | 0.0042 | 0.0008 | 81.0 | Good | Example |
| 33 | 0.050 | 0.024 | 0.76 | 1.26 | 1.5 | 0.059 | 42 | 0.0044 | 0.0008 | 81.8 | Good | Example |

As illustrated in Table 3, in the test levels in which the amount of Al supplied within 10 minutes after start of the LF processing is in the range represented by formula (5), the value of [sol.Al]₃ at the end of the LF processing was within the standard and the desulfurization ratio was higher. In the test levels in which the amount of Al supplied within 10 minutes after start of the LF processing was larger than the range represented by formula (5), the value of [sol.Al]₃ at the end of the LF processing exceeded the upper limit value of the standard. Dealuminization was, thus, necessary in the next process RH and the processing time in the RH was, thus, extended.

### [Fifth example]

Molten pig iron tapped from a blast furnace was subjected to the desiliconization processing, the desulfurization processing, and the dephosphorization processing. The processed molten pig iron was, then, charged into a converter to be subjected to the decarburization refining. As a result, obtained was approximately 250 tons of molten steel having a carbon concentration ranging from 0.05 to 0.09 mass%, a sulfur concentration ranging from 0.0041 to 0.0044 mass%, and a phosphorous concentration ranging from 0.004 to 0.010 mass%. After tapping, the converter slag flowed in a ladle was not discharged. Metallic Al, quicklime, lightly calcined dolomite, and aluminum dross were added into the ladle, and the ladle was transferred to the LF facility illustrated in FIG. 1. The LF processing used quicklime satisfying that the quicklime has a particle diameter equal to or smaller than 20 mm and the sum of the volumes of pores having a pore diameter ranging from 0.5 to 10 µm is 0.2 mL/g. Metallic Al was added so as to satisfy formula (5) within 10 minutes after start of the LF processing.

Table 4 illustrates the sulfur concentrations (chemical analysis values) before and after the desulfurization processing and the desulfurization ratios in respective desulfurization tests. The desulfurization evaluation "Good" means that the sulfur concentration in molten steel after the desulfurization processing was equal to or smaller than 0.0024%.

**Table 4**

| Test No. | Oxygen concentration | Al loss in processing (Air entrainment) | [S]Component change | | | Desulfurization evaluation | Remarks |
|---|---|---|---|---|---|---|---|
| | | | Before Processing [S] | After Processing [S] | Desulfurization ratio | | |
| - | % | kg/t | Mass [%] | Mass [%] | [%] | - | |
| 34 | 20 | 0.50 | 0.0042 | 0.0014 | 66.7 | Good | Example |
| 35 | 18 | 0.47 | 0.0043 | 0.0014 | 67.4 | Good | Example |
| 36 | 16 | 0.45 | 0.0041 | 0.0013 | 68.3 | Good | Example |
| 37 | 14 | 0.37 | 0.0042 | 0.0012 | 71.4 | Good | Example |
| 38 | 12 | 0.32 | 0.0042 | 0.0011 | 73.8 | Good | Example |
| 39 | 10 | 0.30 | 0.0044 | 0.0010 | 77.3 | Good | Example |

As illustrated in Table 4, in the test levels (test numbers 37 to 39) in which the oxygen concentration in ladle is equal to or smaller than 15%, it was found that the Al loss in processing was reduced. The Al loss in processing (air entrainment) was obtained by using the following formula (7).${X}_{A l - loss} = \left({\left[sol.Al\right]}_{2}-{\left[slol.Al\right]}_{3}\right) \times 10 + {W}_{A l - all} - {X}_{A l - l o s s - D e - S} - {X}_{A l - l o s s - slag}$
[*sol.Al*]₂ *: Al concentration (mass%) in molten steel after tapping from converter,*
[*sol.Al*]₃ *: Al concentration (mass%) in molten steel after completion of ladle desulfurization processing,*
*W_{Al-all} : amount (kg*/*t) of Al supplied in ladle desulfurization processing,*
*X_{Al-loss-De-s} : amount (kg*/*t) of Al lost by desulfurization reaction (3CaO* + *3S* + *2Al → 3CaS* + *Al₂O₃),*
*X_{Al-loss-slag}* : *amount (kg*/*t) of Al lost by reduction reaction (6MnO* + *4Al → 2Al₂O₃* + *6Mn, for example) of oxide in slag,*
*X_{Al-loss} : amount (kg*/*t) of Al lost by air entrainment*

### Industrial Applicability

The invention can provide the desulfurization processing method of molten steel and the desulfurization agent that can efficiently perform the desulfurization processing without using CaF₂ and pre-melt flux. Reference Signs List

- 1: LF facility

- 2: ladle
- 3: lid
- 4: electrode
- 5, 6: submerged lance
- 7, 8: bottom-blowing porous brick
- 9: molten steel
- 10: slag
- 11: row material supply chute
- 12: Ar gas introduction pipe

## Claims

1. A desulfurization processing method of molten steel, comprising:
adding a desulfurization agent containing quicklime into a ladle holding the molten steel tapped from a converter; and
stirring the molten steel in the ladle to reduce a sulfur concentration in the molten steel, wherein
the desulfurization agent contains quicklime, where a sum of volumes of pores having a pore diameter ranging from 0.5 µm to 10 µm, inclusive of 0.5 µm and 10 µm, in the quicklime is equal to or larger than 0.1 mL/g;
the quicklime contains particles, where 90% or more of the particles contained in the quicklime has a particle diameter ranging from 1 mm to 30 mm, inclusive of 1 mm and 30 mm;
and
the sum of volumes of pores is obtained as described in the description.

2. A desulfurization agent comprising quicklime, where a sum of volumes of pores having a pore diameter ranging from 0.5 µm to 10 µm, inclusive of 0.5 µm and 10 µm, in the quicklime is equal to or larger than 0.1 mL/g, wherein the quicklime contains particles, where 90% or more of the particles contained in the quicklime has a particle diameter ranging from 1 mm to 30 mm, inclusive of 1 mm and 30 mm, and the sum of volumes of pores is obtained as described in the description.

3. The desulfurization processing method of molten steel according to claim 1, wherein the stirring is performed so as to satisfy a stirring power density represented by the following formula (1): $ε = 6.183 \times \frac{Q \times {T}_{1}}{W} \times \left(ln\left(1+\frac{h}{1.02 \times {10}^{- 4} \times P}\right)+\left(1-\frac{{T}_{g}}{{T}_{l}}\right)\right) \geq 100$
ε *: stirring power density(W*/*t) of gas stirringmoltensteel,*
*Q* : *gas flow rate (Nm³*/*min)*
*W* : *moltensteel amount(t),*
*Tₗ : moltensteel* temperature (°*C*),
*T_{g} : gas* temperature *(°C),*
*h : bath depth(m), P : ambientpressure(Pa)*

4. The desulfurization processing method of molten steel according to claim 1 or 3, wherein an amount of aluminum supplied into the molten steel within 10 minutes after start of the desulfurization processing, the desulfurization processing starting after the molten steel is tapped from a converter, satisfies the following formula (2): $\left({\left[sol.Al\right]}_{1}-{\left[sol.Al\right]}_{2}+0.05\right) \leq {W}_{Al} \leq \left({\left[sol.Al\right]}_{1}-{\left[sol.Al\right]}_{2}+0.1\right)$
[*sol.Al*]₁ *: Al concentration standard upper limit (mass%) in steel grade to be manufactured by being melted*
[*sol.Al*]₂ *: Al concentration (mass%) in molten steel after tapping from converter*
*W_{Al} : amount (kg*/*t) of Al supplied within 10 minutes after start of ladle desulfurization processing*

5. The desulfurization processing method of molten steel according to any one of claims 1, 3 and 4, wherein a flow rate of argon gas blown into the ladle satisfies that a value of πL²/4Q is in a range from 50 to 150 (m/min), where L is the diameter (m) of the ladle and Q is the flow rate of Ar gas *(Nm³*/*min),* such that an oxygen concentration in the ladle is equal to or smaller than 15%.

6. Use of a desulfurization agent in desulfurization of molten steel, wherein the desulfurization agent comprises quicklime, where a sum of volumes of pores having a pore diameter ranging from 0.5 µm to 10 µm (inclusive of 0.5 µm and 10 µm) in the quicklime is equal to or larger than 0.1 mL/g, wherein the quicklime contains particles, where 90% or more of the particles contained in the quicklime has a particle diameter ranging from 1 mm to 30 mm (inclusive of 1 mm and 30 mm) and the sum of volumes of pores is obtained as described in the description,
wherein the desulfurization agent is added into a ladle holding the molten steel which is subsequently stirred so that a sulfur concentration therein is reduced.

7. The use according to claim 6, wherein the stirring is performed so as to satisfy a stirring power density represented by the following formula (1): $ε = 6.183 \times \frac{Q \times {T}_{1}}{W} \times \left(ln\left(1+\frac{h}{1.02 \times {10}^{- 4} \times P}\right)+\left(1-\frac{{T}_{g}}{{T}_{l}}\right)\right) \geq 100$
ε *: stirring power density(W*/*t) of gas stirringmoltensteel,*
*Q* : *gas flow rate (Nm³*/*min)*
*W* : *moltensteel amount(t),*
*Tₗ : moltensteel* temperature *(°C),*
*T_{g} : gas* temperature *(°C),*
*h : bath depth(m), P : ambientpressure(Pa)*

8. The use according to claim 6 or 7, wherein an amount of aluminum supplied into the molten steel within 10 minutes after start of the desulfurization processing, the desulfurization processing starting after the molten steel is tapped from a converter, satisfies the following formula (2): $\left({\left[sol.Al\right]}_{1}-{\left[sol.Al\right]}_{2}+0.05\right) \leq {W}_{Al} \leq \left({\left[sol.Al\right]}_{1}-{\left[sol.Al\right]}_{2}+0.1\right)$
[*sol.Al*]₁ *: Al concentration standard upper limit (mass%) in steel grade to be manufactured by being melted*
[*sol.Al*]*₂ : Al concentration (mass%) in molten steel after tapping from converter*
*W_{Al} : amount (kg*/*t) of Al supplied within 10 minutes after start of ladle desulfurization processing*

9. The use according to any one of claims 6 to 8, wherein a flow rate of argon gas blown into the ladle satisfies that a value of πL²/4Q is in a range from 50 to 150 (m/min), where L is the diameter (m) of the ladle and Q is the flow rate of Ar gas *(Nm³*/*min),* such that an oxygen concentration in the ladle is equal to or smaller than 15%.

## Patentansprüche

1. Verfahren zur Entschwefelungsbehandlung von geschmolzenem Stahl, umfassend:
das Zugeben eines Entschwefelungsmittels, das Branntkalk enthält, in eine Pfanne, die den von einem Konverter abgezapften geschmolzenen Stahl hält; und
das Rühren des geschmolzenen Stahls in der Pfanne, so dass die Schwefelkonzentration in dem geschmolzenen Stahl verringert wird, worin
das Entschwefelungsmittel Branntkalk enthält, wobei eine Summe der Volumen an Poren mit einem Porendurchmesser im Bereich von 0,5 µm bis 10 µm, einschließlich 0,5 µm und 10 µm, in dem Branntkalk gleich oder größer als 0,1 mL/g beträgt;
der Branntkalk Teilchen enthält, wobei 90% oder mehr der in dem Branntkalk enthaltenen Teilchen einen Teilchendurchmesser im Bereich von 1 mm bis 30 mm, einschließlich 1 mm und 30 mm, aufweisen; und
die Summe der Volumen an Poren wie in der Beschreibung beschrieben erhalten wird.

2. Entschwefelungsmittel, das Branntkalk umfasst, wobei eine Summe der Volumen an Poren mit einem Porendurchmesser im Bereich von 0,5 µm bis 10 µm, einschließlich 0,5 µm und 10 µm, in dem Branntkalk gleich oder größer als 0,1 mL/g beträgt, worin der Branntkalk Teilchen enthält, wobei 90% oder mehr der in dem Branntkalk enthaltenen Teilchen einen Teilchendurchmesser im Bereich von 1 mm bis 30 mm, einschließlich 1 mm und 30 mm, aufweisen und die Summe der Volumen an Poren wie in der Beschreibung beschrieben erhalten wird.

3. Verfahren zur Entschwefelungsbehandlung von geschmolzenem Stahl gemäß Anspruch 1, worin das Rühren so durchgeführt wird, dass
eine durch die nachfolgende Formel (1) dargestellte Rührleistungsdichte erfüllt wird: $ε = 6,183 \times \frac{Q \times {T}_{l}}{W} \times \left(ln\left(1+\frac{h}{1,02 \times {10}^{- 4} \times P}\right)+\left(1-\frac{{T}_{g}}{{T}_{l}}\right)\right) \geq 100$
*ε: Rührleistungsdichte (W*/*t) des Gasrührens von geschmolzenem Stahl*
*Q: Gasflussrate (Nm³*/*min)*
*W: Menge geschmolzener Stahl (t)*
*Tₗ: Temperatur geschmolzener Stahl (°C)*
*T_{g}: Gastemperatur (°C)*
*h: Wannentiefe (m) , P: Umgebungsdruck (Pa)*

4. Verfahren zur Entschwefelungsbehandlung von geschmolzenem Stahl gemäß Anspruch 1 oder 3, worin eine Menge an in den geschmolzenen Stahl zugeführtem Aluminium innerhalb von 10 Minuten nach dem Beginn der Entschwefelungsbehandlung, wobei die Entschwefelungsbehandlung beginnt nachdem der geschmolzene Stahl von einem Konverter abgezapft wurde, die nachfolgende Formel (2) erfüllt: $\left({\left[sol.Al\right]}_{1}-{\left[sol.Al\right]}_{2}+0,05\right) \leq {W}_{Al} \leq \left({\left[sol.Al\right]}_{1}-{\left[sol.Al\right]}_{2}+0,1\right)$
[*sol.Al*]₁*: Al-Konzentrationsstandard-Obergrenze (Massen-%) in durch Schmelzen herzustellender Stahlqualität*
[*sol.Al*]₂*: Al-Konzentration (Massen-%) im geschmolzenen Stahl nach dem Abzapfen vom Konverter*
*W_{Al}: Menge (kg*/*t) an innerhalb von 10 Minuten nach dem Beginn der Pfannenentschwefelungsbehandlung zugeführtem Al*

5. Verfahren zur Entschwefelungsbehandlung von geschmolzenem Stahl gemäß einem der Ansprüche 1, 3 und 4, worin eine Flussrate an in die Pfanne geblasenem Argongas erfüllt, dass ein Wert von πL²/4Q in einem Bereich von 50 bis 150 (m/min) liegt, wobei L für den Durchmesser (m) der Pfanne steht und Q für die Flussrate des Ar-Gases *(Nm³*/*min)* steht, so dass die Sauerstoffkonzentration in der Pfanne gleich oder kleiner als 15% beträgt.

6. Verwendung eines Entschwefelungsmittels bei der Entschwefelung von geschmolzenem Stahl, worin das Entschwefelungsmittel Branntkalk umfasst, wobei eine Summe der Volumen an Poren mit einem Porendurchmesser im Bereich von 0,5 µm bis 10 µm (einschließlich 0,5 µm und 10 µm) in dem Branntkalk gleich oder größer als 0,1 mL/g beträgt, worin der Branntkalk Teilchen enthält, wobei 90% oder mehr der in dem Branntkalk enthaltenen Teilchen einen Teilchendurchmesser im Bereich von 1 mm bis 30 mm (einschließlich 1 mm und 30 mm) aufweisen und die Summe der Volumen an Poren wie in der Beschreibung beschrieben erhalten wird,
worin das Entschwefelungsmittel in eine Pfanne gegeben wird, die den geschmolzenen Stahl hält, der anschließend gerührt wird, so dass die Schwefelkonzentration darin verringert wird.

7. Verwendung gemäß Anspruch 6, worin das Rühren so durchgeführt wird, dass eine durch die nachfolgende Formel (1) dargestellte Rührleistungsdichte erfüllt wird: $ε = 6,183 \times \frac{Q \times {T}_{l}}{W} \times \left(ln\left(1+\frac{h}{1,02 \times {10}^{- 4} \times P}\right)+\left(1-\frac{{T}_{g}}{{T}_{l}}\right)\right) \geq 100$
*ε: Rührleistungsdichte (W*/*t) des Gasrührens von geschmolzenem Stahl*
*Q: Gasflussrate (Nm³*/*min)*
*W: Menge geschmolzener Stahl (t)*
*Tₗ: Temperatur geschmolzener Stahl (°C)*
*T_{g}: Gastemperatur (°C)*
*h: Wannentiefe (m), P: Umgebungsdruck (Pa)*

8. Verwendung gemäß Anspruch 6 oder 7, worin eine Menge an in den geschmolzenen Stahl zugeführtem Aluminium innerhalb von 10 Minuten nach dem Beginn der Entschwefelungsbehandlung, wobei die Entschwefelungsbehandlung beginnt nachdem der geschmolzene Stahl von einem Konverter abgezapft wurde, die nachfolgende Formel (2) erfüllt: $\left({\left[sol.Al\right]}_{1}-{\left[sol.Al\right]}_{2}+0,05\right) \leq {W}_{Al} \leq \left({\left[sol.Al\right]}_{1}-{\left[sol.Al\right]}_{2}+0,1\right)$
[*sol.Al*]₁: *Al-Konzentrationsstandard-Obergrenze (Massen-%) in durch Schmelzen herzustellender Stahlqualität*
[*sol.A*l]₂: *Al-Konzentration (Massen-%) im geschmolzenen Stahl nach dem Abzapfen vom Konverter*
*W_{Al}: Menge (kg*/*t) an innerhalb von 10 Minuten nach dem Beginn der Pfannenentschwefelungsbehandlung zugeführtem Al*

9. Verwendung gemäß einem der Ansprüche 6 bis 8, worin eine Flussrate an in die Pfanne geblasenem Argongas erfüllt, dass ein Wert von πL²/4Q in einem Bereich von 50 bis 150 (m/min) liegt, wobei L für den Durchmesser (m) der Pfanne steht und Q für die Flussrate des Ar-Gases *(Nm³*/*min)* steht, so dass die Sauerstoffkonzentration in der Pfanne gleich oder kleiner als 15% beträgt.

## Revendications

1. Procédé de traitement de désulfuration d'acier fondu, comprenant :
l'addition d'un agent de désulfuration contenant de la chaux vive à l'intérieur d'une poche de coulée contenant l'acier fondu soutiré à partir d'un convertisseur ; et
l'agitation de l'acier fondu dans la poche de coulée pour réduire une concentration de soufre dans l'acier fondu, dans lequel
l'agent de désulfuration contient de la chaux vive, où une somme des volumes de pores présentant un diamètre de pores allant de 0,5 µm à 10 µm, y compris de 0,5 µm et de 10 µm, dans la chaux vive est égale ou supérieure à 0,1 mL/g ;
la chaux vive contient des particules, où 90 % ou plus des particules contenues dans la chaux vive présentent un diamètre particulaire allant de 1mm à 30 mm, y compris de 1 mm et de 30 mm; et
la somme des volumes de pores est obtenue comme décrit dans la description.

2. Agent de désulfuration comprenant de la chaux vive, où une somme des volumes de pores présentant un diamètre de pores allant de 0,5 µm à 10 µm, y compris de 0,5 µm et de 10 µm, dans la chaux vive est égale ou supérieure à 0,1 mL/g, dans lequel la chaux vive contient des particules, où 90 % ou plus des particules contenues dans la chaux vive présentent un diamètre particulaire allant de 1 mm à 30 mm, y compris de 1 mm et de 30 mm, et la somme des volumes de pores est obtenue comme décrit dans la description.

3. Procédé de traitement de désulfuration d'acier fondu selon la revendication 1, dans lequel l'agitation est effectuée de manière à satisfaire à une densité d'énergie d'agitation représentée par la formule suivante (1) : $ε = 6,183 \times \frac{Q \times {T}_{l}}{W} \times \left(ln\left(1+\frac{h}{1,02 \times {10}^{- 4} \times P}\right)+\left(1-\frac{{T}_{g}}{{T}_{l}}\right)\right) \geq 100$
ε: *densité d'énergie d'agitation (W*/*t) de gaz agitant de l'acier fondu,*
Q *: débit de gaz (Nm³*/*min),*
*W: quantité d'acier fondu (t),*
*Tₗ: température de l'acier fondu (°C),*
*T_{g}: température du gaz (°C),*
*h : profondeur du bain (m), P : pression ambiante (Pa)*

4. Procédé de traitement de désulfuration d'acier fondu selon la revendication 1 ou 3, dans lequel une quantité d'aluminium fournie à l'intérieur de l'acier fondu dans les 10 minutes après le démarrage du traitement de désulfuration, le traitement de désulfuration démarrant après le soutirage de l'acier fondu à partir d'un convertisseur, satisfait à la formule suivante (2) : $\left({\left[sol.Al\right]}_{1}-{\left[sol.Al\right]}_{2}+0,05\right) \leq {W}_{Al} \leq \left({\left[sol.Al\right]}_{1}-{\left[sol.Al\right]}_{2}+0,1\right)$
[*sol.Al*]₁ *: limite supérieure standard de concentration d'Al* (% *en masse) de la qualité d'acier à fabriquer par fusion*
[*sol.Al*]₂ *: concentration d'Al* (% *en masse) dans l'acier fondu après soutirage à partir du convertisseur*
*W_{Al}: quantité (kg*/*t) d'Al fournie dans les 10 minutes après démarrage du traitement de désulfuration de poche de coulée* (2)

5. Procédé de traitement de désulfuration d'acier fondu selon l'une quelconque des revendications 1, 3 et 4, dans lequel un débit de gaz argon soufflé à l'intérieur de la poche de coulée satisfait au fait qu'une valeur de πL²/4Q se situe dans une plage de 50 à 150 (m/min), où L est le diamètre (m) de la poche de coulée et Q est le débit de gaz Ar *(Nm³*/*min),* de sorte qu'une concentration d'oxygène dans la poche de coulée soit égale ou inférieure à 15 %.

6. Utilisation d'un agent de désulfuration dans la désulfuration d'acier fondu, dans laquelle l'agent de désulfuration comprend de la chaux vive, où une somme des volumes de pores présentant un diamètre de pores allant de 0,5 µm à 10 µm (y compris de 0,5 µm et de 10 µm) dans la chaux vive est égale ou supérieure à 0,1 mL/g, dans laquelle la chaux vive contient des particules, où 90 % ou plus des particules contenues dans la chaux vive présentent un diamètre particulaire allant de 1 mm à 30 mm (y compris de 1 mm et de 30 mm) et la somme des volumes de pores est obtenue comme décrit dans la description,
dans laquelle l'agent de désulfuration est ajouté à l'intérieur d'une poche de coulée contenant l'acier fondu qui est ensuite agitée de sorte qu'une concentration de soufre y soit réduite.

7. Utilisation selon la revendication 6, dans laquelle l'agitation est effectuée de manière à satisfaire à une densité d'énergie d'agitation représentée par la formule suivante (1) : $ε = 6,183 \times \frac{Q \times {T}_{l}}{W} \times \left(ln\left(1+\frac{h}{1,02 \times {10}^{- 4} \times P}\right)+\left(1-\frac{{T}_{g}}{{T}_{l}}\right)\right) \geq 100$
ε: *densité d'énergie d'agitation (W*/*t) de gaz agitant de l'acier fondu,*
Q *: débit de gaz (Nm³*/*min),*
*W: quantité d'acier fondu (t),*
*Tₗ: température de l'acier fondu (°C),*
*T_{g}: température du gaz (°C),*
*h : profondeur du bain (m), P: pression ambiante (Pa)*

8. Utilisation selon la revendication 6 ou 7, dans laquelle lequel une quantité d'aluminium fournie à l'intérieur de l'acier fondu dans les 10 minutes après le démarrage du traitement de désulfuration, le traitement de désulfuration démarrant après le soutirage de l'acier fondu à partir d'un convertisseur, satisfait à la formule suivante (2) : $\left({\left[sol.Al\right]}_{1}-{\left[sol.Al\right]}_{2}+0,05\right) \leq {W}_{Al} \leq \left({\left[sol.Al\right]}_{1}-{\left[sol.Al\right]}_{2}+0,1\right)$
[*sol.Al*]₁ *: limite supérieure standard de concentration d'Al* (% *en masse) de la qualité d'acier à fabriquer par fusion*
[*sol.Al*]₂ *: concentration d'Al* (% *en masse) dans l'acier fondu après soutirage à partir du convertisseur*
*W_{Al}: quantité (kg*/*t) d'Al fournie dans les 10 minutes après démarrage du traitement de désulfuration de poche de coulée*

9. Utilisation selon l'une quelconque des revendications 6 à 8, dans laquelle un débit de gaz argon soufflé à l'intérieur de la poche de coulée satisfait au fait qu'une valeur de πL²/4Q se situe dans une plage de 50 à 150 (m/min), où L est le diamètre (m) de la poche de coulée et Q est le débit de gaz Ar *(Nm³*/*min),* de sorte qu'une concentration d'oxygène dans la poche de coulée soit égale ou inférieure à 15 %.
